

July 1, 1930.

R. D. PIKE

1,769,605

PROCESS FOR MAKING ELECTROLYTIC IRON

Filed March 13, 1926



## UNITED STATES PATENT OFFICE

ROBERT D. PIKE, OF PIEDMONT, CALIFORNIA

## PROCESS FOR MAKING ELECTROLYTIC IRON

Application filed March 13, 1926. Serial No. 84,454.

My present invention relates to a process for making electrolytic iron from leach liquors in non-diaphragm cells, and includes a leaching process whereby iron and/or copper is dissolved by the action of ferric iron on metallic iron and/or copper ores; and the iron dissolved from the metallic iron and/or copper ores and that used for removing copper and other metals (if present) from solution, is deposited electrolytically in a cell without diaphragms, but having insoluble anodes; such deposition of iron resulting in the regeneration of the liquor for further leaching operations.

Under conditions known hitherto, if iron were to be plated out of solutions in electrolytic cells with insoluble anodes, it has been necessary to employ diaphragms to separate the anolyte from the catholyte, if commercial current efficiencies were to be obtained. This is because of the well-known fact, based upon the principles of electro-chemistry, that ferric iron in contact with a cathode will be reduced to ferrous iron before metallic iron can be plated out. This is explained electro-chemically by the following equations:



These equations show that deposition of iron cannot occur theoretically when  $\text{Fe}^{+++}$  is in contact with the cathode.

I have found in practice that if the electrolytic iron cell with insoluble anodes be run at 70° centigrade or above, with ferrous chloride leach solutions containing about 12% Fe, even small percentages of ferric iron as low as 1% in the catholyte will seriously lower current efficiency. These are the conditions substantially obtaining in my former applications, Serial Numbers 58,012, 58,009 and 58,010 (all filed September 23, 1925) and Serial Number 87,509, filed February 11, 1926, in all of which inventions I employ diaphragm cells and keep the concentration of  $\text{Fe}^{++}$  substantially below .05%.

I have discovered that if I employ as the electrolyte a solution of ferrous chloride containing preferably about 12% iron in a non-diaphragm cell with an insoluble anode of

the type hereafter described, at about room temperature, and use a current density of preferably 7 amperes per square foot, and operate the cell so that the effluent contains about .75%  $\text{Fe}^{+++}$ , the current efficiency is from 80% to 85% and the cell voltage with 1½-inch electrode spacing is about 1.75 volts. These conditions are realized by employing a cell in which the incoming electrolyte is fed in at the top of the bath and the outflowing leach liquor containing about .75% ferric iron is removed from the bottom of the bath—this condition being necessary because I have found that the ferric iron, as formed, tends to flow naturally toward the bottom of the cell.

It is possible to employ wide variation in the concentration and composition of the electrolyte, in the current density and temperature employed, without departing from the scope of my invention. For example, in practice the electrolyte will tend to assume a temperature of from 20° to 30° centigrade, or a little above actual room temperature, and this is satisfactory, although I have found it to be a general rule that the effect of  $\text{Fe}^{+++}$  in lowering current efficiency becomes the more pronounced the higher the temperature; and on this account, if it is desirable, as is sometimes the case, to heat the leach solutions for promoting extraction of metals, the reduced liquors should be cooled by spraying or other suitable device before returning to the electrolytic iron cells.

If sponge iron or iron scrap is the raw material employed it is unnecessary to heat the leach solutions to promote efficient extraction; but if the raw material is a sulphide mineral, such, for example, as chalcoelite, bornite, or even chalcopyrite, the leach solutions should be heated, and in the case of the last-mentioned mineral, to boiling. Some other sulphide minerals, notably galena (lead sulphide), are more easily decomposed by relatively cold dilute solutions of ferric chloride. A preferable method for proceeding is to make sponge iron from copper and precious metal bearing cinders from pyrite roasters. The leaching of such iron is so conducted, as described hereafter, as to effect

a complete separation of the iron from the more noble metals, i. e., copper, silver, and gold; and these last-named are recoverable as valuable by-products.

5 In the accompanying drawing,

The figure illustrates a flow sheet for production of electrolytic iron from sponge iron. With slight modifications, as described below, this flow sheet may be applied to the treatment of any of the materials above mentioned.

10 It will be understood that there may be considerable variation from the described flow sheet; as, for example, in the composition of the leach solutions and the manner of their application, without departing from my invention, and also that diaphragm cells may be employed, if desired.

15 Referring in detail to the drawing, return 20 leach from the electrolytic tank house, containing about 12% total iron as chloride, of which about .75% is ferric iron, and at a temperature of 20° to 30° centigrade, enters the agitator 1, where it meets the underflow from 25 the thickener 2, as well as the clarified liquor from the filter 3. The discharge from agitator 1 goes to thickener 4, the underflow of which goes to filter 3. The cake from filter 3 is the exhausted tails free from iron, copper, and other metals which the original 30 sponge iron may have contained.

35 The overflow from thickener 4 is pumped by pump 5 to agitator 6, where it meets the underflow from thickener 7. Agitator 6 discharges into thickener 2. The overflow from thickener 2 goes to agitator 8, where it meets the fresh sponge iron, and the agitator 8 discharges into thickener 7. The overflow from thickener 7 is completely reduced copper-free electrolyte. The system described 40 of thickeners 2, 4, 7 and agitators 1, 6, 8, is in effect a counter-current leach arrangement in which the fresh sponge iron completes reduction of the leach, and the fresh leach completes solution of the iron.

45 However, the sponge iron may contain copper and/or other metals which are electro-negative to iron; and such metals may be completely dissolved in agitator 1, and 50 completely precipitated in agitator 8. They will therefore accumulate in the leaching system. To counteract this tendency, a portion of the overflow from thickener 4 is "bled" to agitator 9, where sufficient sponge iron is 55 added to precipitate all of the copper and other metals electro-negative to iron. Agitator 9 discharges into thickener 10, the underflow of which passes to filter 11, the cake of which is principally cement copper and 60 may contain other metals. The clear liquor from filter 11 returns to agitator 9. The overflow from thickener 10 joins that from thickener 7.

65 The full flow of electrolyte is next treated in a tank 12 with H<sub>2</sub>S to precipitate traces of Zn,

and other relative electro-positive metals. The sulphide precipitate is removed in thickener 13 and filter 14. A discard may then be made, if desired, to take care of accumulation of such elements as Ca, Mg, Al, and alkalies, if these be present. The discard, if made, is replaced with fresh ferrous chloride.

70 The electrolyte next goes to supply tank 15, and thence through electrolytic tank cells 16. These are of the type hereinafter described. 75 The anodes are preferably of plate graphite, and the cathodes steel sheets with oxidized surfaces to facilitate stripping of the electrolytic iron. The current density is preferably 7 amperes per square foot, and the cell voltage about 1.75. The regenerated leach goes to tank 17 and pump 18 returns it to agitator 1.

80 In treating chalcocite, or other sulphide mineral, the same flow sheet is employed as in Fig. 1 except that the mineral, instead of sponge iron, is introduced into the agitator 8. With sulphide mineral there will be no appreciable accumulation of copper in the counter-current system, and all of the copper will be in solution in the overflow of thickener 7. This entire overflow will therefore pass through the copper cementation system 85 9, 10, 11, and this system will receive no liquor from any other point in the counter-current system. After precipitating the copper and/or other relatively noble metals, the liquor passes to the tank 12, and thence on 90 through the cycle as before.

95 The leach liquor may be heated by any suitable means (not shown), on its way from the electrolytic iron cells to agitator 1, and if heating is employed, at any point in the cycle a corresponding cooling means such as a spray pond, or other suitable device (not shown), should be employed, so as to deliver 100 the electrolyte in a relatively cool condition to supply tank 15.

105 Having thus described my invention, what I claim as new and desire to secure by Letters Patent is:

110 1. The process of making substantially copper-free electrolytic iron from copper-bearing metallic iron which consists in dissolving the latter in a counter-current leaching apparatus with a leach liquor containing ferric iron; "bleeding" a portion of the liquor from a point in the counter-current system, treating this bled portion with sufficient metallic iron to completely reduce the ferric iron in solution and completely precipitate copper in 115 solution, then passing the completely reduced and copper-free liquor discharged from this step, together with the reduced copper-free liquor from the counter-current leach, to electrolytic cells for the deposition of iron and the regeneration of the leach.

120 2. The process of making substantially copper-free electrolytic iron from copper-bearing metallic iron which consists in dissolving the latter in a counter-current leaching appa- 125

ratus with a leach liquor containing ferric iron, "bleeding" a portion of the liquor from a point in the counter-current system, treating this bled portion with sufficient metallic iron to completely reduce the ferric iron in solution and completely precipitate copper in solution, then passing the completely reduced and copper-free liquor discharged from this step, together with the reduced copper-free liquor from the counter-current leach, to the top of non-diaphragm cells for the deposition of iron and the regeneration of the leach and withdrawing the regenerated solution from the bottom of the cells.

ROBERT D. PIKE.

15

20

25

30

35

40

45

50

55

60

65